

# UNITED STATES PATENT OFFICE.

JOHN D. PRINCE, OF BOSTON, MASSACHUSETTS.

## LEATHER SUBSTITUTE.

1,305,621.

Specification of Letters Patent.

Patented June 3, 1919.

No Drawing.

Application filed July 22, 1916. Serial No. 110,698.

*To all whom it may concern:*

Be it known that I, JOHN D. PRINCE, a citizen of the United States, and resident of Boston, in the county of Suffolk and State 5 of Massachusetts, have invented a new and useful Improvement in Leather Substitutes, of which the following is a specification.

This invention relates to a sheet material designed to be used as a substitute for 10 leather, buckskin, chamois, and the like, and also as a substitute for rubber in many of its applications. It is particularly directed to the industry of manufacturing boots, shoes and the like, but it is of such a nature 15 as to have a very wide range of usefulness; some other applications which I may mention being floor coverings, upholstery, vehicle tops and covers, waterproof clothing, piston packing, etc.

20 One of the particular features of advantage of this invention is the fact that it has a permanent fibrous appearance, so that it may, from the point of view of looks, fully satisfy the requirements of a substitute for 25 leather, buckskin, chamois, or other material of the same general nature. In this respect my material is sharply distinguished from rubber compounds, which have been in use, inasmuch as the latter have, at the beginning 30 and throughout their life, a glossy appearance as contrasted with a fibrous one.

Again, my material may be used by shoe manufacturers in exactly the same manner 35 as leather is used today, no matter whether it be applied as soles, heels, or uppers. The very same machinery, dies, models and other appliances may be used. It is also susceptible to the same finishing process, including 40 the polishing, coloring, edging and stitching, whether the latter be known as the channeling method, the McKay method, the stitched aloft method, the stitched down method, or any of the other well known methods of securing soles to uppers.

45 Furthermore, this material is about 20% cheaper than high grade leather, and on grinding tests, it has shown its wearing qualities to be 85% greater than that of the best scoured oak sole leather, and 73% better 50 than the rubber compounded soles, such as are in ordinary use.

The material is about 100% more flexible than leather of corresponding thickness; it is waterproof, although it absorbs a sufficient amount of moisture to make it more 55 desirable than rubber, particularly when applied to the manufacture of shoes or waterproof clothing, for the reason that it does not produce the so-called sweating effect. It will not slip on wet pavements, 60 nor will it adhere to clothing. It is much more resilient than leather, so that it is applicable to use in place of the so-called rubber heels, for the purpose of avoiding jars and shocks. It is heat proof and cold proof. 65

With this brief outline of the general nature and characteristics of the material, I will proceed to describe the manner in which it is made.

Broadly considered, the material is composed of a fiber which has been ground so as to be broken into short lengths, and rubber compounded with sulfur; the whole being suitably vulcanized into the desired sheet form and thickness. Other ingredients which are added in compounding the material serve to enhance its valuable qualities; and, in the best form of the invention now known to me, the same is composed of 70 cotton fiber, selected sheet Ceylon rubber, 75 pure rubber gum, known as concho, reclaimed rubber or shoddy, pontianak, pulverized magnesia, red oxid of iron, and sulfur.

I find cotton fiber to be the most desirable 85 of all, owing to its strength and availability, but, other vegetable fibers, such, for instance, as hemp, flax, jute, sisal, wood fiber, straw or grasses, may be employed.

In carrying out the invention, the cotton, 90 as it is baled, is provided and subjected to a grinding process; *e. g.*, between heavy rollers in a machine commonly known as a "rag mill," which is designed for grinding fibrous material. The cotton is preferably 95 ground in mass so that the grinding process shortens instead of crushing the fiber, the effect being a tearing apart as distinguished from a flat pressure. The cotton is ground to lengths of approximately 1/100 100 of an inch and is then ready for use in compounding my material. Thus, when I say

in the claims "short length" fiber, I refer to fibers of not more than about one to ten one hundredths of an inch long.

To a batch aggregating approximately 20 pounds, the ingredients mentioned are mixed in substantially the following proportions:

4 $\frac{1}{2}$  pounds of cotton fiber, in its ground condition;

10 1 $\frac{1}{2}$  pounds of selected sheet Ceylon rubber;

1 $\frac{1}{2}$  pounds of pure Concho rubber gum;

9 $\frac{1}{2}$  pounds of reclaimed rubber or shoddy;

15 1 pound of pontianak;

$\frac{1}{4}$  pound of pulverized magnesia;

$\frac{1}{3}$  pound red oxid of iron; and

1 $\frac{1}{4}$  pounds sulfur.

These ingredients are compounded and thoroughly milled between heated rollers into a mass, as is customary in compounding rubber, which is well understood in the art.

I prefer to use the selected sheet Ceylon rubber because it is very strong, clean and pure. However, other kinds of rubber can be used in its place, such, for instance, as up-river Para.

The Concho rubber is selected because of its great adhesiveness and elasticity. Furthermore, it is a good, pure rubber and blends well with the other ingredients incorporated. But, in this case also, other rubber gums can be used, such, for instance, as Manocoba.

The pontianak, which is a byproduct of a resin, is particularly desirable owing to its adhesive properties, but other resins may be used in its place.

40 The reclaimed rubber, which is commonly referred to as shoddy, is a regular ingredient of rubber compounds, and is desirable for the purpose of cheapening the product.

45 The pulverized magnesia is, as is well understood, a drier, and is generally used in rubber mills. It has a sufficient drying effect, is light in weight and a good filler. In place of it some such material as chalk 50 flour could be used, if desired.

55 The red oxid of iron is used for the purpose of a coloring agent, but it could be substituted by any other well known pigment material, such as lamp black, black carbon, chrome yellow, yellow ochre, Indian red, etc.

The sulfur is, as will be well understood, for the purpose of vulcanization.

After the mixture has been compounded and milled as described, it may be vulcanized in any of the ordinary ways, such for instance, as in a flat surface press, or on rolls wrapped with wet cloth. A very convenient way is to vulcanize it in a press, the 60 plates of which are blocked apart a sufficient

distance to give the finished sheet material the desired thickness. The vulcanization is preferably carried out at a temperature equivalent to 35 pounds steam pressure, and for a time period of 25 minutes. This quick 70 vulcanization, at a comparatively low temperature, is very desirable from the point of view of economy of time, fuel and labor, and it also is advantageous as it minimizes the tendency of the heat of vulcanization 75 to injure the natural oily or waxy material in the cotton fiber. The manner of vulcanizing will be well understood to any one skilled in the art, without further description.

80 After vulcanization, either one or both surfaces of the material may be buffed to remove any glossy appearance resulting from the action of the plates in the vulcanizer, so as to provide a natural, fibrous appearance. This buffing may be accomplished by any of the ordinary methods 85 commonly employed in rubber manufactures, and is well understood in the art.

90 Instead of simply vulcanizing the material into sheets, it may be associated with cloth, such, for instance, as duck or sheeting, by calendering, in a well known manner, the composition onto one or both surfaces 95 of the cloth. The cloth thus calendered with the material, may be subjected to heat for the purpose of vulcanization, after which it may be applied to such uses as waterproof clothing, uppers for shoes, upholstering or other cases where a very flexible leather or 100 rubber sheet is required.

Without setting forth at greater length the characteristics and advantages of my invention, I may repeat that two of its greatest features of value lie in the fact that 105 it may be employed by the manufacturer in exactly the same way that leather is used, and that it has, at the beginning, and during its whole life, a fibrous leathery appearance.

110 In conclusion, it will be understood that various changes may be made in the ingredients and proportions specified; and in the method of treating, compounding and vulcanizing the various substances, without departing from the spirit and scope of my 115 invention; hence I do not intend to be limited to details hereinbefore described except as they may be specifically included in the claims.

120 What I claim is:—

1. A permanently fibrous material designed as a substitute for leather and the like, comprising short length fiber, a pure, clean rubber, and a strong and adhesive rubber, the same being compounded with sulfur 125 and vulcanized.

2. A permanently fibrous material designed as a substitute for leather and the like, comprising a short length fiber, a pure, clean rubber, a strong and adhesive rubber, 130

- a resin, and a drying agent, the whole being compounded with sulfur and vulcanized.
3. A permanently fibrous material designed as a substitute for leather and the like, comprising a short length fiber, a pure, clean rubber, a strong and adhesive rubber, shoddy, a resin, a drying agent, and a pigment, the same being compounded with sulfur and vulcanized.
4. A permanently fibrous material designed as a substitute for leather and the like, comprising short length fiber, selected sheet Ceylon rubber, gum Concho, shoddy,
- pontianak, magnesia, red oxid of iron, and sulfur, in substantially the proportions specified, the whole being vulcanized.
5. A permanently fibrous material designed as a substitute for leather and the like, comprising short length fiber, selected sheet Ceylon rubber, gum Concho, shoddy, 20 pontianak, magnesia, red oxid of iron and sulfur, the whole being vulcanized.

In testimony that I claim the foregoing as my invention I have signed my name this 20th day of July, 1916.

JOHN D. PRINCE.